

## UNITED STATES PATENT OFFICE.

MORTON ROLAND SHERBINO, OF DETROIT, MICHIGAN, ASSIGNOR TO HYDRAULIC BRAKE COMPANY, OF DETROIT, MICHIGAN, A CORPORATION OF CALIFORNIA.

## NONCORROSION SOLUTION.

No drawing.

Application filed March 19, 1926. Serial No. 96,084.

This invention relates to a solution comprising castor oil, alcohol and a phosphorous compound soluble in alcohol, the solution being used primarily, although not necessarily, as the fluid medium of a hydraulic braking system for automobiles.

Heretofore, it has been common practice to use a solution of alcohol and castor oil in substantially equal proportions for actuating the pistons in so-called hydraulic braking systems, such for example as shown in the patent to Malcolm Loughead, No. 1,531,798 of March 31st, 1925. This solution has been used because of the fact that castor oil thus dissolved in alcohol has no detrimental effect upon rubber used for cup washers and for piping, and at the temperatures encountered in practice has a sufficiently constant viscosity for practical purposes. It has been found in practice that even chemically pure castor oil, when mixed with either ethyl or methyl alcohol brings about a gradual corrosion of the commonly used metals, such as iron, steel, brass, copper, and the metals found in die casting alloys.

I have found that the corrosion of the above named metals is greatly decreased by the addition to the castor oil-alcohol solution of a compound of phosphorous, and that these compounds have no detrimental effect upon the rubber of the hose or cup washers used in the system. I have found particularly that tri-sodium phosphate ( $Na_3PO_4 \cdot 12H_2O$ ) successfully diminishes this corrosion. The quantity of tri-sodium phosphate used for successfully minimizing the corrosion is about one-half gram per gallon of solution, but the amount may be increased to any amount which can be successfully dissolved in the alcohol.

One of the forms of corrosion which has given rise to trouble in the operation of fluid operated vehicle brakes, is the copper sulphide which forms as a result of the presence of sulphur in the rubber with which the brake solution comes in contact and the presence of copper in the tube which conducts the brake solution to the work cylinders. This copper sulphide forms along the interior of the copper tubing, creating a thin scale which, through vibration of the tubing, becomes dislodged and is carried by

the solution into the brake cylinders where it eventually lodges between the rubber cup and the cylinder wall, causing abrasion of the rubber and leakage of the fluid.

I believe that the compound of phosphorous acts as a negative catalytic agent, which very materially slows down the action of the dissolved sulphur upon the copper. I believe, further, that the same negative catalytic action is responsible for the diminution of the corrosion of other metals which come into contact with the brake fluid.

Although my invention has been described for use in a fluid braking system, it is equally applicable to any other system making use of a solution of castor or other oil in alcohol.

I claim:

1. A solution of castor oil in alcohol, rendered non-corrosive by the addition of an alkali metal phosphate.
2. A solution of castor oil in alcohol, rendered inert and non-corrosive by the addition of a small proportion of tri-sodium phosphate.
3. A solution of castor oil in alcohol, rendered inert and non-corrosive by the addition of a small proportion of a sodium phosphate.
4. A solution for use in fluid braking systems, comprising substantially equal parts of castor oil and alcohol and substantially one-half gram of an alkali metal phosphate to one gallon of the alcohol-castor oil solution.
5. A brake solution comprising alcohol, an oil soluble in alcohol, and an alkali metal salt containing phosphorous.
6. The combination with a liquid medium, comprising a castor oil and alcohol solution, in contact with metallic copper and vulcanized rubber, of an alkali metal phosphate held in solution by the medium.
7. A liquid medium for fluid actuated braking systems which comprise metal and sulphur-containing vulcanized rubber in contact with the medium, the medium comprising a solution of castor oil and alcohol with a small portion of a salt containing phosphorous in solution therewith for minimizing the corrosion of the metal by the sulphur.

8. In a fluid system exposed both to copper and to sulphur-containing vulcanized rubber, the combination therewith of a liquid medium including alcohol and castor oil, and means for preventing the corrosion of the copper by the sulphur, comprising a small portion of a salt containing phosphorous in solution with the alcohol.
9. The process of minimizing the corrosion of copper by the sulphur in vulcanized rubber, which consists in covering the area of copper exposed to the sulphur with a liquid

medium containing castor oil, alcohol, and an alkali metal phosphate.

10. The combination with a solution of 15 castor oil in alcohol and small amounts of sulphur, of means for minimizing the corrosion of metallic copper with which the solution comes into contact, comprising a small portion of a salt containing phosphorous held in the solution.

In witness whereof, I hereunto subscribe my name this 2nd day of March, 1926.

MORTON ROLAND SHERBINO.